# EUROPEAN PATENT SPECIFICATION

(11) **EP 0 949 371 B1**
(45) Date of publication and mention of the grant of the patent: **05.11.2008**
(21) Application number: 99108935.0
(22) Date of filing: 16.09.1996
(51) Int. Cl.: D04H 1/42, D04H 1/54, D04H 1/48, D04H 3/14, D04H 3/10

(54) **Filament nonwoven fabrics and method of fabricating the same**
Vliesstoffe von Filamentfäden und Verfahren zur Herstellung
Etoffes non tissées de filaments et méthode de fabrication

(30) Priority: 29.09.1995 JP 25167995; 03.10.1995 JP 25607995; 03.10.1995 JP 25608095; 03.10.1995 JP 25608395
(43) Date of publication of application: 13.10.1999
(62) Divisional of application: 96114791.5
(73) Proprietor: UNITIKA LTD., Amagasaki-shi Hyogo-ken (JP)
(72) Inventor: Nagaoka, Koichi, c/o Research and Development Center of UNITIKA LTD., Kyoto-fu (JP); Matsuoka, Fumio, c/o Research and Development Center of UNITIKA LTD., Kyoto-fu (JP); Ichise, Naoji, c/o Research and Development Center of UNITIKA LTD., Kyoto-fu (JP)
(74) Representative: Kügele, Bernhard

(56) References cited:
- EP-A- 0 530 987
- EP-A- 0 597 427
- EP-A- 0 637 641
- DATABASE WPI Section Ch, Week 199442 Derwent Publications Ltd., London, GB; Class A23, AN 1994-338776 XP002272638 & JP 06 264343 A (TOYOBO KK) 20 September 1994 (1994-09-20)
- DATABASE WPI Section Ch, Week 9435 Derwent Publications Ltd., London, GB; Class A23, AN 94-283801 XP002023666 & JP 06 212511 A (UNITIKA LTD) 2 August 1994 (1994-08-02)

## Description

### FIELD OF THE INVENTION

The present invention relates generally to filament nonwoven fabrics which are degradable due to microorganisms and the like in natural environments and a method of manufacturing the same. More particularly, the invention relates to a degradable filament nonwoven fabric which can be produced from a biodegradable polymer composed principally of a thermoplastic aliphatic polyester under particular conditions, and a method of manufacturing the same.

### BACKGROUND OF THE INVENTION

Hitherto, nonwoven fabrics which are degradable due to microorganisms have been known including, for example, biodegradable nonwoven fabrics made from natural or regenerated filaments, such as cotton, flax, hemp, ramie, wool, rayon, chitin, and alginic acid filaments.

However, such degradable nonwoven fabrics, which are generally hydrophilic and water absorptive, are not suitable for use in such an application as disposable diaper top sheet, wherein- it is required that the fabric be hydrophobic and less water absorptive and should have a dry feel when it gets wet. Another problem is that such nonwoven fabrics are very much liable to deterioration in strength and dimensional stability under wet environmental conditions; and this has limited the possibility, of exploiting new uses for such nonwoven fabrics in general industrial material applications. Further, such nonwoven fabrics, because of their non-thermoplastic nature, have no thermoformability and are therefore less processable.

Recently, therefore, research and development efforts have been positively made for microbially degradable filaments which may be obtainable by the melt spinning technique from a microbially degradable polymer having thermoplastic and hydrophobic characteristics, and microbially degradable nonwoven fabrics made up of such filaments. In particular, a group of polymers generally called aliphatic polyesters are attracting high attention because they have microbial degradation characteristics. Specifically, such polymers include, for example, poly-β-hydroxyalkanoate as represented by microbially degradable polyester, poly-ω-hydroxyalkanoate as represented by polycaprolactone, polyalkylene dicarboxylate composed of a polycondensate of glycol and dicarboxylic acid, such as polybutylene succinate, or copolymers of these polymers. In such situation, and with recent development of a new polymerization process which can efficiently produce polymers of high polymerization degree, various attempts have been made to produce filaments from poly-α-oxyacid, a polymeric product as represented by poly-L-lactic acid, and nonwoven fabrics comprised of such filaments. Of aforesaid aliphatic polyesters, polylactic acid in particular has a relatively high melting point such that, when a nonwoven fabric comprised of that material would prove to be very useful in applications which require heat resistance. As such, much expectation is now entertained for possibilities of polylactic nonwoven fabrics for practical use.

A polylactic nonwoven fabric is already disclosed in JP-A-7-126970 in which is described a staple filament nonwoven fabric composed principally of polylactic acid. In JP-A-6-212511 there is given a teaching about a polylactic staple filament material useful for the manufacture of polylactic staple filament nonwoven fabrics. However, the manufacture of such a staple filament nonwoven fabric involves many operating stages, from melt spinning and up to nonwoven fabric forming; and this poses a problem from the standpoint of production cost economy.

Whilst, in a number of publications, including JP-A-7-48769, JP-A-6-264343, International Nonwovens Journal, Vol. 7, No. 2, pp 69 (1995), and EP 0637641 (A1), suggestions are given for fabrication of filament nonwoven fabrics from polylactic acid under the so-called spun bond technique in which filaments are extruded by melt extrusion for being formed into webs deposited on a screen. However, in JP-A-7-48769, a suggestion is simply given that a nonwoven fabric can be produced from polylactic acid-based polymers by employing the spun bond technique, with no particular mention made as to any specific process for fabrication of such a fabric and the properties of the nonwoven fabric to be obtained. In JP-A-6-264343, which pertains to a biodegradable agricultural filament assembly, there is no detailed statement as to such important manufacturing conditions as filament drafting speed, and other necessary particulars, nor is there any teaching on the properties of the nonwoven fabric produced. The teaching of International Nonwovens Journal, Vol. 7, No. 2, pp 69 (1995) is merely such that hard and brittle plate-like, polylactic spun bonded fabrics were obtained. In EP 0637641 (A1), there is no teaching that a polylactic spun bonded fabric having good flexibility and high mechanical strength can be produced.

### DISCLOSURE OF THE INVENTION

The present invention is intended to solve the foregoing problems and has as its primary object the provision of a filament nonwoven fabric degradable due to microorganisms and the like in natural environments and yet having sufficient mechanical strength for practical use.

In order to accomplish this object, according to the present invention there is provided a nonwoven fabric made up of filaments comprised of a biodegradable polymer composed principally of a polylactic acid-based polymer or a polyalkylene dicarboxylate, wherein the filaments are partially bonded with heat and pressure or the filaments are three-dimensionally-entangled af ter partially bonded wi th heat and pressure and wherein the filaments have a crystallization degree of from 7 to 40 % and a supercool index of 0.4 or more.

Further, according to the present invention, there is provided a method of fabricating a nonwoven fabric made up of filaments comprised of a biodegradable polymer composed principally of a polylactic acid-based polymer or polyalkylene dicarboxylate, which comprises the steps of melting the biodegradable polymer, said biodegradable polymer having a melt flow rate of 10 to 100 g/10 minutes as measured at 190°C according to ASTM-D-1238 (E), in a temperature range of from (Tm + 20)°C to (Tm + 80)°C, where Tm°C is the melting point of the biodegradable polymer; extruding the melt through a spinneret into filaments; drafting the extruded filaments by means of a suction device disposed below the spinneret under a quenching air blow generated through a conventional quenching device at a drafting speed of from 1,000 to 5,000 m/minute, thereby fining them down into finer filaments; then depositing such filaments, as they are spread open each other, and are laid up on a travelling collector surface to form a web; and heat treating the web thereby to obtain the nonwoven fabric.

In this way, the nonwoven fabric in accordance with the present invention is formed from filaments obtained through the process of rapid filament quenching beneath the spinneret and filament drafting at a drafting speed of from 1,000 to 5,000 m/minute, the filaments having a crystallization degree of from 7 to 40 % and a supercool index of 0.4 or more. This ensures good flow behavior during the process of thermoforming, especially when the thermoforming operation involves complex and acute-angled shaping. Moreover, the nonwoven fabric exhibits less torsion stress and high breaking extension at thermoforming temperatures. This provides an advantage that any breakage which would otherwise possibly occur at times of thermoforming can be effectively prevented. Further, since the nonwoven fabric has a three-dimensional entangled structure, various types of thermoformed products of such a filament nonwoven fabric have a larger specific surface area than thermoformed articles of known sheet materials and can be composted in a very short time. At the same time, this feature enables the filament nonwoven fabric of the invention to find its way into the markets for formed products of which air/liquid permeability is required, as well as those of which fibrous or nonwoven fabric-like hand is required.

### BRIEF DESCRIPTION OF THE DRAWINGS

Figs. 1 through 6 are illustrations showing, by way of example, different cross-sectional configurations of constituent filaments of nonwoven fabrics in accordance with the present invention.

### DETAILED DESCRIPTION OF THE INVENTION

Filaments employed in the present invention are preferably comprised of a polylactic acid-based polymer.

For the polylactic acid-based polymer is used a polymer having a melting point of 100°C or more selected from the group consisting of poly(D-lactic acid), poly(L-lactic acid), copolymers of D-lactic acid and L-lactic acid, copolymers of D-lactic acid and hydroxy-carboxylic acid, and copolymers of L-lactic acid and hydroxy-carboxylic acid, the selected polymer having a melting point of 100°C or more, or a blend of such polymers.

Where a homopolymer such as poly(D-lactic acid) or poly(L-lactic acid) is used as a polylactic acid-bashed polymer, it is desirable that a plasticizer be added thereto especially for enhancement of spinnability during the process of spinning and flexibility improvement with respect to the resulting filaments and nonwoven fabric. Examples of useful plasticizers for such purposes include triacetin, lactic acid oligomers, and dioctyl phthalate. The amount of addition of such a plasticizer should be from 1 to 30 % by weight, preferably from 5 to 20 % by weight.

Where the polylactic acid-based polymer is a copolymer of lactic acid and hydroxy-carboxylic acid, examples of hydroxy-carboxylic acid include glycolic acid, hydroxybutanoic acid, hydroxyvaleric acid, hydroxypentanoic acid, hydroxycaproic acid, hydroxyheptanoic acid, and hydroxyoctanoic acid. Of these, hydroxycaproic acid or glycolic acid is particularly preferred from the standpoints of microbial degradation performance and cost economy.

The above enumerated polylactic acid-based polymers may be used alone or in the form of a blend of two or more kinds. In case that such polymers are used in the form of a blend, conditions such as polymers to be mixed and mixing proportions may be suitably determined in consideration of spinnability and other factors.

Such polymers each may be added with various additives, such as dulling agent, pigment, and crystallizing agent, as required within the limits in which the advantageous feature of the invention will not be affected.

The cross section of each constituent filament of the nonwoven fabric may have any cross-sectional configuration, such as solid and otherwise. More specifically, it is preferable that the filament has one of such cross-sectional configurations as hollow section, odd-shaped section, sheath-core type composite section, and slit type composite section.

Fig. 1 shows a cross sectional view in which filament 1 has a hollow cross section. Reference numeral 2 designates a filament portion, and 3 designates a hollow portion. Where a nonwoven fabric is made up of filaments having such a hollow section, the nonwoven fabric has good degradation capability. The reason is that as microorganisms and moisture erode inward from the outer circumferential portion for entry into the hollow portion 3 through holes formed in the filament portion 2 so that the surface area per unit polymer weight is so enlarged as to enhance the rate of degradation by microorganisms and the like. Further, it is significant to note that a filament having an hollow section exhibits good performance for enhancement of quenching efficiency with respect to filaments spun, because per-unit-time polymer passage through a quenching region during spinning operation is relatively small in weight terms, and because the filament contains therein air bubbles of a small specific heat.

Where the filament has a polygonal odd-shaped cross section or a planar odd-shaped cross section as shown in Figs. 2 and 3, such sectional configuration can enhance filament quenching and spreading-open efficiency in the spinning stage, and can provide improved degradability with respect to the nonwoven fabric to be obtained. The reason for this is that where a filament has an odd-shaped sectional configuration, the filament provides a larger surface area per unit polymer weight.

In case that the filament cross section is a sheath-core type composite section, it is important that after at least one of a polylactic acid-based polymer and a blend of plural kinds of polylactic acid-based polymers is chosen as one filament component, filaments of a sheath-core structure be formed of two kinds of components including the one filament component, the two kinds of components being arranged in such a manner that one having a higher melting point (hereinafter referred to as high melting point component) is used to assume a core position, the other of a lower melting point (hereinafter referred to as low melting point component) being used to assume a sheath position. In this case, it is also important that between the two components there must be a melting point difference of at least 5°C or more, preferably 10°C or more, more preferably 20°C or more. It is to be noted, however, that where two or more kinds of polylactic acid-based polymer blends are used as core component(s) and/or sheath component(s), the melting point difference between the core and sheath components is determined in such a manner that for the core component, the melting point of one of the constituent polymers of the blend which has a lowermost melting point is taken as a basis, whereas for the sheath component, the melting point of one of the constituent polymers of the blend which has the highest melting point is taken as a basis. Through this arrangement, for the purpose of bonding a web with heat and pressure, it is possible to carry out such bonding operation at a comparatively low temperature, say at a temperature close to the melting point of the sheath component, without causing fusion to the high melting point component of the core portion. Therefore, the resulting nonwoven fabric can have good flexibility.

In case that the filament cross section is a split type composite section, a nonwoven fabric formed from filaments of such a cross-sectional configuration can exhibit good degradability and good flexibility. The term "split type composite section" used herein refers to a filament section such that the filament comprises two kinds of filament components arranged in divisions separate from one another in a circumferential direction of the filament section, the two kinds of filament components including at least one of a polylactic acid-based polymer and a blend of plural kinds of polylactic acid-based polymers, chosen as one filament component, wherein both components extend continuously in the longitudinal direction of the filament and are exposed to the exterior of the filament. Specifically, cross-sectional configurations as shown in Figs. 4 to 6 may be exemplified. More particularly, Fig. 4 shows a cross section wherein two components of filament 1, that is, high melting point component 4 and low melting point component 5 have respective radially extending divisions arranged in alternate relation. Fig. 5 shows a cross section wherein low melting point component 5 constitutes a center portion of filament 1 and wherein high melting point component 4 has a plurality of divisions arranged along a circumferential edge of the low melting point component 5 in such a way that they protrude outward of the low melting point component 5. According to these cross sectional filament configurations, division of the filament itself is accelerated as a portion of a component having higher degradability (usually, low melting point component) is degraded. Therefore, a nonwoven fabric formed from filaments of such cross-sectional configuration will have improved degradability. In Fig. 6, there is shown a filament cross section which is similar to the one shown in Fig. 4 but is different in that there is provided an hollow portion 3. Such filament configuration provides for further improvement in degradability, and filament quenching and spreading-open efficiency. Where such split type composite section is used, it is possible as well to carry out fusion bonding in a temperature range near the melting point of low melting point component 5 during the process of web bonding with heat and pressure. In this operation, no fusion is caused to high melting point component 4. Thus, it is possible to obtain a nonwoven fabric having good flexibility.

In addition to the above described cross-sectional filament configurations, various other odd-shaped composite cross-sectional configurations may be used including, for example, triangular, quadrangular, hexagonal, planar, Y-shaped, and T-shaped.

In the manufacture of the filament nonwoven fabric of the invention, a web is partially bonded with heat and pressure without individual filaments being joined at intersection points, so that the web can retain a sheet-like configuration of nonwoven structure. Such a nonwoven fabric has good flex properties because the constituent filaments are bonded only in partially formed fusion-bonded areas.

In the manufacture of the filament nonwoven fabric of the invention, filaments are previously partially bonded with heat and pressure, whereby filaments are enabled to temporarily retain a web form for purposes of subsequent three-dimensionally entangling. As a result, the nonwoven fabric obtained can have improved shape retention and improved dimensional stability. At such partially effected temporary bonded areas with heat and pressure, filaments are separated entirely or at least partially by a subsequent entangling treatment, so that filaments including the separated filaments can make up a three-dimensional entanglement formation. Thus, the fabric obtained possesses such mechanical strength and dimensional stability as can meet the requirements for practical use. Additionally, the fabric retains larger parts of non-fusion-bonded areas and can, therefore, also have good flexibility.

Next, the method of fabricating a nonwoven fabric of polylactic acid-based polymer filaments in accordance with the present invention will be explained.

The nonwoven fabric of the invention can be efficiently manufactured by the so-called spun bond process. A polylactic acid-based polymer of the above mentioned type having a melt flow rate of 10-100 g/10 minutes as measured at a temperature of 190°C in accordance with ASTM-D-1238 (E) is melted in a spinning temperature range of from (Tm + 20)°C to (Tm + 80)°C, where Tm°C is the melting point of the polymer, and the melt is spun into filaments through a spinneret which provides a desired filament cross section. The filaments obtained are quenched by means of a conventional quenching device known in the art, such as horizontal blow type or annular blow type, and then the filaments are drafted by a suction device, such as air sucker, in an air stream of from 1,000 to 5,000 m/min. to the desired fineness. Masses of filaments discharged from the suction device are spread open each other and then deposited while being spread open each other on a travelling collector device, such as a screen conveyor, being thus formed into a web. Then, the web formed on the travelling collector device is subjected to heat treatment. A nonwoven fabric is thus obtained.

In melt spinning operation, as earlier mentioned, the polymer used should be melted within a temperature range of from (Tm + 20)°C to (Tm + 80)"C, where Tm°C is the melting point of the polymer. However, where a blend of two or more kinds of polylactic acid-based polymers is used, Tm °C should be a melting point which is the highest of the melting points of the constituent polymers of the blend. If the spinning temperature is lower than (Tm + 20) °C, drafting operation in high-speed air currents will be of low efficiency. If the spinning temperature is higher than (Tm + 80) °C, some delay will occur in the process of crystallization at the quenching stage, resulting in inter-filament fusion and poor spreading effect, as well as some thermal decomposition of the polymer itself. Therefore, it is difficult to obtain a nonwoven fabric having good flexibility and uniform texture.

In the process of drafting filaments by means of a suction device to a desired fineness, as already stated, it is important that the drafting speed be within the range of from 1,000 to 5,000 m/min. The drafting speed may be suitably selected according to the MFR value of the polymer. If the drafting speed is less than 1,000 m/min., oriented crystallization of the polymer is retarded, which may result in inter-filament adhesion; and therefore the resulting nonwoven fabric is likely to have hard feel and inferior mechanical strength. If the drafting speed is more than 5,000 m/min., the process of drafting is forced to be carried out in excess of a critical drafting limit, and this results in filament break occurrences, it being thus difficult to maintain stable operation.

For heat treatment of webs, a partial bonding apparatus with heat and pressure is used to give partial bonding with heat and pressure at a temperature lower than the melting point which is the lowest of the melting points of polymeric components of the filament. The expression "partially bonding with heat and pressure" means formation of fusion bonded areas by embossing or ultrasonic fusion bonding. Specifically, a web is passed through a clearance between a heated embossing roll and a flat surface metal roll for formation of inter-filament fusion bonded areas.

More particularly, individual bonded areas with heat and pressure, as particular partial areas in a web, each have an area of 0.2 to 15 mm² which may be of any configuration, such as circular, elliptic, diamond, triangular, T-shaped, and number sign-shaped. Preferably, the density of distribution of such areas, that is, the density of bonded areas with heat and pressure is within the range of 4 to 100 bonded areas per cm². If the density of bonded areas with heat and pressure is less than 4 bonded areas per cm², no improvement can be had in the mechanical strength and shape retention capability of the resulting nonwoven fabric. If the density is more than 100 bonded areas per cm², the resulting nonwoven fabric is rough and hard and has only poor flexibility. The ratio of total bonded area with heat and pressure to total surface area of the web, that is, pressure bonded area ratio, should be 3 to 50 %, though it depends upon the area of each individual pressure bonded area. If the pressure bonded area ratio is less than 3 %, the resulting nonwoven fabric cannot have improved mechanical strength or improved form retention capability. If the pressure bonded area ratio is more than 50 %, the resulting nonwoven fabric is rough and hard and has only poor flexibility.

Operating temperature for bonding with heat and pressure, that is, the surface temperature of the embossing roll, as already stated, must be lower than the melting point of the polymer used. However, where the web to be bonded with heat and pressure is formed from filaments comprised of a blend of two or more kinds of polylactic acid-based polymers, or where the web is formed from bicomponent filaments having a composite cross-sectional configuration, for example, such a sheath-core type composite section or a split type composite section as earlier mentioned, the melting point of one polymer whose melting point is the lowest of those of all component polymers of the blend, or the melting point of one component of the bicomponent composite cross section which is lower than that of the other is taken as a reference, and operation must be carried out at an operating temperature lower than such a melting point. If the operating temperature exceeds that temperature limit, there may occur polymer adhesion to the bonding apparatus with heat and pressure, with the result that operating efficiency is adversely affected. In addition, the resulting nonwoven fabric has a very hard hand, it being thus impractical to obtain a reasonably flexible nonwoven fabric.

For the operation of bonding with heat and pressure, in addition to the earlier mentioned method using heated embossing rolls, it is possible to adopt a method such that an ultrasonic fusion bonding apparatus is employed to ultrasonically apply a high frequency to the web on a pattern roll, thereby to form inter-filament fusion bonded areas in a pattern section. More specifically, the ultrasonic fusion bonding apparatus comprises an ultrasonic oscillator having a frequency of about 20 kHz which is generally called "horn", and a pattern roll having raised projections arranged circumferentially thereon in a area pattern or belt-like pattern. The pattern roll is disposed below the ultrasonic oscillator so that partial hot fusion bonding can be effected by passing a web through a nip between the ultrasonic oscillator and the pattern roll. Raised projections arranged on the pattern roll may be of a single row or plural rows. In the case of plural-row arrangement, the raised projections may be arranged either in parallel rows or in staggered rows. -

Above said operation of partially bonding with heat and pressure using embossing rolls or such an ultrasonic fusion bonding apparatus may be carried out either in a continuous process or in a separate stage. Either way of operation may be suitably selected according to the intended use of the nonwoven fabric.

Next, in the case of a nonwoven fabric of the invention wherein the nonwoven fabric includes area-like fusion bonded areas which are formed as a result of partial separation by a three-dimensionally entangling treatment of individual filaments at previously formed partial temporary bonded areas with heat and pressure, or wherein individual filaments at previously formed partial temporary bonded areas with heat and pressure are already completely separated and individual filaments in non-fusion-bonded areas are three-dimensionally entangled together so that all constituent filaments are integrated as an integral unity, the manufacturing method is as described below.

In this case, a web formed on the travelling deposition apparatus in manner as earlier described is subjected to partial bonding with heat and pressure by a partial bonding apparatus with heat and pressure in an operating temperature range of from (Tm - 80)°C to (Tm - 50)°C, where (Tm)°C represents the melting point of one component polymer which is the lowest of the melting points of all component polymers of the filaments of the web, with linear pressure of a roll set within the range of from 10 to 100 kg/cm, whereby temporary bonded areas with heat and pressure are formed. Next, by effecting a three-dimensionally entangling treatment, individual filaments at temporary bonded areas with heat and pressure at least partially separated so that all constituent filaments including the filaments in separated condition are three-dimensionally entangled into an integral unity. Thus, a filament nonwoven fabric can be obtained.

In this way, by previously effecting partial bonding with heat and pressure, it is possible to permit temporary shape retention so as to enhance the shape retention and mechanical strength of the web for subsequent three-dimensionally entangling operation, thereby facilitating process handling in that operation. Further, since individual filaments at the partial temporary bonded areas with heat and pressure are at least partially separated so that a final nonwoven fabric retains the greater part of its area in non-fusion-bonded condition, it is possible to obtain a nonwoven fabric having good flexibility. In case that all the individual filaments at partial temporary bonded areas with heat and pressure are completely separated by three-dimensionally entangling treatment, the resulting nonwoven fabric has very good flexibility while retaining its nonwoven configuration in order. Whilst, in case that separation is not completely effected, with temporary heat bonded areas partially left unremoved, three-dimensional entanglement of constituents filaments including separated filaments provides dimensional stability and mechanical strength and, in addition, the fusion bonded areas remaining unremoved serve to provide some reinforcing effect in respect of dimensional stability and mechanical strength.

Aforesaid previously formed partial bonded areas with heat and pressure are preferably such that individual bonded areas with heat and pressure have an area of 0.2 to 15 mm², with the density of fusion bonded areas therein being 4 - 100 bonded areas per cm², preferably 5 - 80 bonded areas per cm². If the density of fusion bonded areas is less than 4 bonded areas per cm², any improvement cannot be obtained in mechanical strength and configurational retention property of the web after heat / pressure bonding. If the density exceeds 100 bonded areas per cm², the processability of the web for three-dimensional entangling treatment is unsatisfactory. The pressure bonded area ratio is 3-50 %, preferably 4-40 %. If the pressure bonded area ratio is less than 3 %, any improvement in dimensional stability cannot be obtained with respect to the resulting nonwoven fabric. Conversely, if the ratio is hither than 50 %, it is likely that the web is less processable for the purpose of three-dimensional entangling.

For bonding operation with heat and pressure, aforesaid conditions of operating temperature and a linear pressure of a roll set are particularly important. If the operating temperature is lower than (Tm - 80)°C and/or if the linear pressure of a roll set is lower than 5 kg/cm, the effect of bonding with heat and pressure is unsatisfactory, and no improvement can be achieved in respect of shape retention performance and dimensional stability of the resulting nonwoven fabric. If the operating temperature is higher than (Tm - 50)°C and/or if the linear pressure of a roll set is higher than 30 kg/cm, the effect of bonding with heat and pressure is excessively large so that individual filaments at the bonded areas with heat and pressure can hardly be partially separated during three-dimensionally entangling operation. Therefore, three-dimensional entanglement of individual filaments in non-fusion-bonded areas cannot sufficiently be effected, it being thus difficult to form all constituent filaments of the web into an integral unity.

By setting conditions of operating temperature and linear pressure of a roll set in such a manner as described above, it is possible to previously form partial temporary bonded areas with heat and pressure within a mass of constituent filaments of the filament web. These partial temporary bonded areas with heat and pressure serve to improve the shape retaining performance and mechanical strength of the web after bonding with heat and pressure and to facilitate process handling during three-dimensional entangling operation. Further, the partial temporary bonded areas with heat and pressure have a certain degree of bonding capability such that individual filaments at such areas can be easily separated at least partially by a mechanical external force applied during the three-dimensionally entangling operation.

The three-dimensional entangling treatment which is given after partial temporary bonding with heat and pressure is carried out through a treatment of pressured liquid stream in which the web is subjected to the action of pressure liquid streams, or through needle punching operation.

Where three-dimensional entangling is carried out through a treatment of pressured liquid stream, a web produced by the earlier mentioned spun bond process, which is formed with partial temporary bonded areas with heat and pressure, is placed on a moving porous support plate and is exposed to the action of pressured liquid streams, whereby individual filaments, including at least partially separated filaments at bonded areas with heat and pressure, are three-dimensionally entangled so that all constituent filaments of the web are integrated as a whole.

To generate pressured liquid streams, an apparatus including an orifice having plural jet holes arranged in one row or plural rows, the jet holes having a bore diameter of from 0.05 to 2.0 mm, preferably from 0.1 to 0.4 mm, adjacent jet holes being 0.3-10 mm spaced apart, is employed. Jet streams of pressured liquid are delivered in a jet pressure range of from 5 to 150 kg/cm² G. If the pressure of liquid streams is less than 5 kg/cm² G, it is difficult to partially separate bonded areas with heat and pressure. Therefore, entangling of constituent filaments cannot be effected to any sufficient extent. If the pressure is higher than 150 kg/cm² G, individual filaments are too densely entangled, and the resulting nonwoven fabric is likely to be less flexible. Jet holes should be arranged in a row along a direction orthogonal to the direction of advance of the web. In case that jet holes are arranged in plural rows, they are preferably arranged in staggered relation from the standpoint of subjecting the web to uniform action of pressured liquid streams. Orifices having jet holes arranged therein may be arranged in plurality. For the pressured liquid, it is common to use fresh water or warm water. The distance between the jet holes and the web should be from 1 to 15 cm. If the distance is less than 1 cm, the texture of the resulting nonwoven fabric is rendered irregular. If the distance is more than 15 cm, the impact force of liquid streams, upon their impingement against the web, is so low that three-dimensional entangling is not sufficiently effected. A support element for supporting the web during pressured liquid treating operation may be, for example, a wire cloth or mesh screen of 10 to 300 mesh, or a porous plate, but is not limited thereto, it being only required that the support element should permit pressured liquid streams to penetrate through the web.

According to the application for which the nonwoven fabric as a final product is to be used, the web subjected to entangling treatment on one side according to the above described method may be turned over and again subjected to entangling treatment by pressured liquid streams. By so doing it is possible to obtain a nonwoven fabric closely integrated on both sides which can exhibit good dimensional stability and high mechanical strength.

After pressured liquid treatment is given, it is necessary that excess moisture be removed from the treated web. For removal of such excess moisture, any known method may be used. For example, it is possible to mechanically remove any residual water to some degree by using a squeezing device, such as mangle roll, and then remove the rest of the water content by employing a dying apparatus, such as continuous hot air drier. Such drying operation may be carried out as ordinary dry heat treatment, but where required, may be carried out as wet heat treatment. For the choice of treating conditions, such as drying temperature and drying time, in carrying out drying operation, conditions may be selected not only for the purpose of moisture removal, but also to allow reasonable degree of shrinkage with respect to the nonwoven web.

Where it is intended to provide three-dimensional entangling by needle punching, a web produced according to the spun bond process, with partial temporary bonded areas with heat and pressure formed thereon, is punched through by punch needles so that filaments including at least partially separated filaments at those areas bonded with heat and pressure are three-dimensionally entangled for integration as a whole.

Needle punching is preferably carried out under the conditions of; needle depth, 5-50 mm; punching density, 50-400 punches/cm². If the needle depth is less than 5 mm, the degree of entanglement of filaments is insufficient, which in turn results in poor dimensional stability, while a needle depth of more than 50 mm poses a problem from the standpoint of productivity. If the punch density is less than 50 punches/cm², constituent filaments at bonded areas with heat and pressure may not be smoothly separated and entangling of filaments may not sufficiently be effected; and the resulting nonwoven fabric may lack dimensional stability. If the punch density is more than 400 punches / cm², filament breaks due to punch needles may occur and the resulting nonwoven fabric may be of lower mechanical strength. Punch needles are selectable in respect of thickness, length, number of barbs, barb pattern. etc. according to the single filament fineness, intended use, etc.

Aforesaid pressured liquid stream treatment is applicable to products of lower weight per unit area (15 - 200 g/m²), and by such treatment it is possible to obtain nonwoven fabrics having good flexibility and high mechanical strength. Needle punch treatment is applicable to products of higher weight per unit area (100 - 500 g/m²), and by such treatment it is possible to obtain having good flexibility, good air permeability, and good water permeability. The reason for selection of applicable treatment according to the weight per unit area is that there is some difference in web penetration capability between pressured liquid streams and needle punches. For example, when a pressured liquid stream treatment is applied to articles of higher weight per unit area, pressured liquid streams do not penetrate through the web in the direction of web thickness; therefore, entangling of filaments is effected only with respect to the surface layer of the web, no uniform three-dimensional entanglement being formed over the entire web. Therefore, it is desirable that which one of the treatment methods is to be selected should be determined according to the weight per unit area of the nonwoven fabric and the purpose for which the nonwoven fabric is to be used.

When selection is made in this way, at fusion bonded areas which have been destroyed through three-dimensionally entangling treatment and still remain as such to some degree, the pressured bonded area density is 20 bonded areas per cm² or less, preferably 10 bonded areas per cm² or less, and the pressure bonded area ratio is 15 % or less, preferably 10 % or less. A filament nonwoven fabric having such fusion bonded areas can take advantage of the presence of non-fusion-bonded areas to effectively provide filament to filament entangling through the three-dimensionally entangling treatment. Thus, the nonwoven fabric can exhibit good dimensional stability and high mechanical strength. In case that fusion bonded areas partially remain in existence, such fusion bonded areas adds to the dimensional stability and mechanical strength of the nonwoven fabric. Further, as earlier mentioned, temporary bonded areas with heat and pressure are separated in part or wholly by three-dimensionally entangling treatment, and this in effect means the presence of a large non-fusion-bonded area, which enables the fabric to exhibit good flexibility, while in non-fusion-bonded region, filaments are three-dimensionally entangled, which adds to dimensional stability and mechanical strength.

According to the invention, as earlier stated, a nonwoven fabric of the invention is comprised of filaments spun from a biodegradable polymer composed principally of a thermoplastic aliphatic polyester, the filaments having a crystallization degree of from 7 to 40 % and a supercool index of 0.4 or more.

According to the present invention, a method of fabricating a nonwoven fabric made up of filaments comprised of a biodegradable polymer composed principally of a thermoplastic aliphatic polyester comprises the steps of melting the biodegradable polymer, said biodegradable polymer having a melt flow rate of from 10 to 100 g/10 minutes as measured at 190°C according to ASTM-D-1238 (E), in a temperature range of from (Tm + 20)°C to (Tm + 80)°C, where Tm°C is the melting point of the biodegradable polymer; extruding the melt through a spinneret into filaments; drafting the extruded filaments by means of a suction device disposed below the spinneret under a quenching air blow generated through a conventional quenching device and at a drafting speed of from 1,000 to 5,000 m/minute, thereby fining them down into finer filaments: then depositing such filaments, as they are spread open each other, and are laid up on a travelling collector surface to form a web; and heat-treating the web thereby to obtain the nonwoven fabric.

As stated above, filaments used in the invention are formed from a biodegradable polymer composed principally of a thermoplastic aliphatic polyester.

Examples of thermoplastic aliphatic polyesters include poly(α-hydroxy acid), such as polyglycolic acid or polylactic acid, ahd copolymers of repeating units mentioned above or constituents of such polymers. Also, polycondensates of glycol and dicarboxylic acid may be mentioned as such, including, for example, polyethylene oxalate, polyethylene succinate, polyethylene adipate, polyethylene azelate, polybutylene oxalate, polybutylene succinate, polybutylene adipate, polybuylene sebacate, polyhexamethylene sebacate, polyneopentyl oxalate, and polyalkylene dicarboxylate copolymer comprising any of these as repeating units.

In the present invention, of the above enumerated, polylactic acid-based polymer, any one of polybutylene succinate, polyethylene succinate, polybutylene adipate, and polybutylene sebacate, or copolymers in which these polymers are included as repeating units are preferred from the standpoints of biodegradability, spinnability or the like.

As stated above, in case that the aliphatic polyester is a polylactic acid-based polymer, specifically, any one of poly(D-lactic acid), poly(L-lactic acid), copolymer of D-lactic acid and L-lactic acid, copolymer of D-lactic acid and hydroxycarboxylic acid, and copolymer of L-lactic acid and hydroxycarboxylic acid which has a melting point of 100°C or more is preferred. In a copolymer of lactic acid and hydroxycarboxylic acid, the hydroxy-carboxylic acid may be, for example, glycolic acid, hydroxybutyric acid, hydroxyvaleric acid, hydroxypentanoic acid, hydroxycaproic acid, hydroxyheptanoic acid, or hydroxyoctanoic acid. In this case, in order that the nonwoven fabric, as a product, may possess good formability, the number-average molecular weight of the polylactic acid-based polymer is preferably 50,000 - 95,000.

In the case where, aliphatic polyester is polyalkylene dicarboxylate, any polymer selected from the group consisting of polybutylene succinate, polyethylene succinate, polybutylene adipate, and polybutylene sebacate, or a copolymer in which such polymers are included as repeating units, is preferred as such. Specifically, a copolymer of not less than 70 mol % of butylene succinate and one of ethylene succinate, butylene adipate, and butylene sebacate is preferred.

Such biodegradable polymers as above enumerated may be used in a blend of plural selected polymers.

Further, it is possible to use, as a biodegradable polymer, a polycondensed product of aforesaid thermoplastic aliphatic polyester and aliphatic polyamide, such as polycapramide (nylon 6), polytetramethylene adipamide (nylon 46), polyhexamethylene adipamide (nylon 66), polyundecanamide (nylon 11), and polylauramide (nylon 12), that is, an aliphatic polyester amide-based copolymer.

From the standpoints of spinnability and resulting filament property, it is desirable that such biodegradable polymer should have a number-average molecular weight of not less than about 20,000, preferably not less than 40,000, more preferably not less than 60,000. Polymers which are chain-extended with a small amount of diisocyanate or tetracarboxylic dianhydride to enhance polymerization degree may also be used.

The biodegradable polymer may be added with various kinds of additives, such as dulling agent, pigment, and crystallizing agent, as required, but within the limits which are not detrimental to the intended effects. In particular, addition of crystallizing agents, such as talc, boron nitride, calcium carbonate, magnesium carbonate, and titanium oxide is desirable, because it can prevent inter-filament blocking at spinning and quenching stages, and because it can enhance crystallization during thermoforming operation and improve heat resistance and mechanical strength characteristics, However, since excessive promotion of filament crystallization will effect formability characteristics, the amount of such addition is within the range of from 0.1 to 3.0 wt %, more preferably from 0.5 - 2.0 wt %.

The filament configuration of constituent filaments of the nonwoven fabric may be solely of aliphatic polyester or may be of a composite of two or more kinds of alphatic polyesters. The filament cross section of constituent filaments may be a usual circular section, an irregular section, an hollow section, or a composite section such as sheath-core type section, as stated above.

The single filament fineness of constituent filaments of the nonwoven fabric is preferably 20 denier or less, more preferably 1 to 12 denier. If the fineness is more than 20 denier, filament quenching at the spinning stage is hindered, and in addition the flexibility characteristics of the resulting nonwoven fabric are unfavorably affected. This is inconvenient from the standpoint of thermoforming operation with the nonwoven fabric, because the fabric does not allow smooth working especially when some complex and acute-angled deformation work is involved.

The weight per unit area of the nonwoven fabric, as a commercial product, is preferably within the range of 10 to 500 g/m². If the weight per unit area is less than 10 g/m², the nonwoven fabric is of poor appearance and insufficient in mechanical strength, being unsatisfactory for practical use. If the weight per unit area is more than 500 g/m², flexibility is affected. Where finer single filament is involved, the fabric is of greater denseness than a nonwoven fabric of the same weight per unit area which is made up of filaments of coarser single filament. However, the fact that deterioration in mechanical strength due to biodegradation is faster must be taken into consideration. Where the mechanical strength of the filament itself is low, a larger weight per unit area is required in order to enable the fabric to maintain a certain degree of strength.

Constituent filaments of the nonwoven fabric of the invention should have a crystallization range of from 7 to 40 % and a supercool index of 0.4 or more. This is basic requirements for affording efficient working during thermoforming operation, especially at the time of complex and acute angle deformation work.

A crystallization degree is determined from a wide-angle X-ray diffraction pattern of powdered filament according to the Ruland method. Whilst, a supercool index is expressed by an equation based on a fusion enareaherm curve (heat up/melting and heat down), details of which will be described hereinafter. These are reference indices as to formability. Where a crystallization degree is less than 7 %, fusion breakage is likely to occur at a high deformation region. If a crystallization degree is more than 40 %, heat deformation is less likely to occur, which makes it difficult to carry out high drafting forming. Where a supercool index is less than 0.4, the nonwoven fabric lacks transformation ability during thermoforming operation.

The above mentioned requirements being met by constituent filaments of the nonwoven fabric means that the nonwoven fabric is acceptable for thermoforming operation with it. This in turn means that strain-stress is low at the thermoforming temperature and elongation at break is high. Therefore, the nonwoven fabric can be prevented from breaking during thermoforming operation. For example, elongation at break of the nonwoven fabric is 20 % or more, preferably 30 % or more, more preferably, 40 % or more.

Another basic requirement is that the filament nonwoven fabric and constituent filaments thereof are not liable to shrink during thermoforming operation. The reason is that if any shrinking of the web sheet occurs at the time of forming, the sheet is taken up by the mold, which prevents stable continuos forming operation. Therefore, the shrinked area of the nonwoven fabric at the time of thermoforming operation is not more than 10%, preferably not more than 5 %, more preferably not more than 2 %.

The nonwoven fabric of the invention maintains a sheet-form configuration having a nonwoven structure because of the fact that the web is subjected to heat treatment.

One configurational feature of the nonwoven fabric of the invention is that the web is partially bonded with heat and pressure. The nonwoven fabric of such configuration in accordance of the invention has good flexibility performance, because the fabric is bonded only at the fusion bonded areas. This provides for maintenance of smooth working capability during thermoforming operation, especially at the time of complex and accute-angled deformation work, and also provides for improvement in the form retention capability of the nonwoven-fabric during thermoforming operation.

Another configurational feature of the nonwoven fabric of the invention is such that the fabric has fusion bonded areas formed when individual filaments at preformed partial temporary bonded areas with heat and pressure were partially separated through three-dimensional entangling treatment, and such that individual filaments at non-fusion-bonded portions in areas other than the fusion bonded areas are three-dimensionally entangled so that the fabric is integrated as a whole.

A still another configurational feature of the nonwoven fabric of the invention is such that individual filaments at preformed partial temporary bonded areas with heat and pressure are completely separated and three-dimensionally entangled through three-dimensional entangling treatment and are integrated as a whole.

Details of these configurations are same as those already described and are not repeated herein.

Next, method of manufacturing above described nonwoven fabric will be explained in detail.

As earlier described, a biodegradable polymer must have an MFR value measured according to the method stated in ASTM-D-1238 (E) which is within the range of 10 - 100 g/10 min. If the MFR value is less than 10 g/10 min., the melt viscosity is too high and therefore the efficiency of drafting by air sucker or the like is poor, which may be a cause of filament break at the spinning stage. If the MFR value is more than 100 g/10 min., the melt viscosity is too low, which leads to poor drafting efficiency, it being thus difficult to carry out operation in stable condition.

Spinning temperature should be suitably selected by taking into consideration the type of polymer, MFR value of the polymer, or the like. If the spinning temperature is too low, the result is poor drafting efficiency. If the spinning temperature is too high, interfilament adhesion may be caused, resulting in poor filament-spreading-out effect; and in addition, thermal decomposition of the polymer itself will proceed.

During spinning operation, filaments just after being spun is subjected to quenching air blow at more than a certain rate with care not to cause any substantial filament shaking. The suction device is preferably set at a location below and at 1 to 2 m distance from the spinneret. Where necessary, earlier mentioned crystallizing agent may be added to enhance quenching effect.

For the purpose of drafting and thinning filaments spun by means of the suction device, as earlier mentioned, it is important that the drafting speed be within the range of 1,000 to 5,000 m / min. Through such arrangement, it is possible to achieve a crystallization degree of from 7 to 40 % with respect to constituent filaments of the nonwoven fabric and a supercool index of 0.4 or more. If the drafting speed is less than 1,000 m/min., crystallization of oriented polymers will not progress so that the crystallization degree of filaments may be less than 7 %, thus resulting in lower mechanical strength of the resulting nonwoven fabric. If the drafting speed is more than 5,000 m/min., crystallization of oriented polymers will progress excessively so that the crystallization degree of filaments may exceed 40 % and, in addition, the supercool index may be lower than 0.4. As a result, the filaments are subject to higher strain-stress at thermal deformation temperatures, which leads to poor thermoformability. Therefore, it is especially preferable that the drafting speed be 1,200 to 3,000 m/min.

For heat treatment of web, it is possible to use partial bonding with heat and pressure which creates fusion bonded areas by embossing treatment or ultrasonic fusion bonding treatment. In this case, the operating temperature for bonding with heat and pressure, that is, the surface temperature of the embossing roll is preferably lower than the melting point of one polymer having lowest melting point in case that the web is comprised of plural kinds of polymers. If the operating temperature exceeds this temperature, polymer adhesion to the bonding apparatus with heat and pressure may occur, which adversely affects operating efficiency. Moreover, the resulting nonwoven fabric feels hard and is less adaptable to a mold having a complex configuration, leading to poor formability.

As stated above, pressure bonded area ratio for bonding with heat and pressure may be from 3 to 50 %. If this ratio is less than 3 %, the resulting fabric will have poor form retention property necessary for fabric handling purposes and poor dimensional stability. If.this ratio is more than 50 %, the resulting nonwoven fabric feels hard and is less adaptable to a mold having a complex configuration, leading to poor formability.

This partial bonding with heat and pressure may be carried out in a continuous process operation or in a separate operation stage. The choice of either method may be determined suitably, for example, according to the formed product to be manufactured using the nonwoven fabric obtained.

Other details of this partial bonding with heat and pressure are as already described. For example, two or more kinds of components comprised of biodegradable polymers are melt spun through a spinneret which provides a composite filament cross section, and partial bonding with heat and pressure is carried out at a temperature lower than the melting point of the polymer which is the lowest in melting point of the two or more kinds of polymers.

Another method for heat treatment of webs is such that temporary bonded areas with heat and pressure are formed by applying a partial bonding treatment with heat and pressure to the web; then individual filaments at the temporary bonded areas with heat and pressure are partially separated by effecting three-dimensional entangling treatment ; then individual filaments in separated state are three-dimensionally entangled into overall integration.

In that case, a partial bonding operation with heat and pressure for forming temporary bonded areas with heat and pressure is carried out by pressing the web by means of the embossing roll. For this purpose, it is important that such bonding operation is carried out at an operating temperature of from (Tm - 80)°C to (Tm - 50)°C, where Tm°C is the melting point of the polymer having the lowest melting point of the component polymers, with the linear pressure of a roll set at 10 - 100 kg/cm. The reason for this is as already stated.

Other details of the three-dimensional entangling treatment are as already stated.

As already stated, it is possible to carry out thermoforming operation using the biodegradable filament nonwoven fabric as a material. In this case, if the component polymer of the nonwoven fabric, or the nonwoven fabric are comprised of plural polymers, one polymer having the highest melting point of the polymers is taken as a subject polymer, and the nonwoven fabric is preheated at a temperature higher than the glass transition temperature of, but lower than the melting point of the subject polymer, being then subjected to pressed forming in a mold. Thereafter, for improving the mechanical strength of the resulting formed piece, crystallization is enhanced at temperatures in the vicinity of the crystallizing temperature.

### EXAMPLES

The invention will be explained more specifically with reference to the following examples. It is understood, however, the invention is in no way limited to these examples.

In the following examples and comparative examples, various property values were determined as stated below.

MFR (Melt Flow Rate) value (g/10 min.): measured at 190°C in accordance with the method described in ASTM-D-1238 (E).

Melting point (°C) and supercool index: In a fusion-endotherm curve based on measurements obtained by means of a differential scanning calorimeter, Model DSC-2 made by Perkin Elmer, with a sample weight of 5 mg, and the rate of temperature rise set at 20°C/min., an intermediate temperature between a shift start temperature at the base line and a shift end temperature was determined to be a glass transition temperature Tg (°C), and a temperature which gives the extreme of enareahermic peaks was determined to be a melting point Tm (°C). Then, after the sample was maintained in melted condition for 10 minutes, quenching was effected at a temperature decreasing rate of 20°C/min. In an exotherm curve obtained, a temperature which gives a maximum value was determined to be a crystallizing temperature Tc (°C). Where two or more maximum values were given, a main peak was adopted as the maximum value. Supercool index was determined according to the following relation. $Supercool index = \left(Tm-Tc\right) / \left(Tc-Tg\right)$

Weight per unit area (g/m²): From each sample in standard condition were prepared 10 specimens, each of 10 cm x 10 cm. After the moisture content of each specimen was brought to equilibrium, each specimen was weighed for determining the weight (g) thereof. The average of the values obtained was converted into a value per unit area, which was defined as weight per unit area (g/m²).

Filament crystallization degree (%): Measured according to a wide-angle X-ray diffraction method (powdered; Ruland Method). In the wide-angle X-ray diffraction method, diffracted X-ray interference intensity measurements were made in the direction of reflection angle 2θ, whereby an diffracted intensity curve was obtained. Then, from the diffracted intensity curve were separated to a crystal-based diffracted peak and an amorphous portion-based dispersion halo, which were quantitatively determined. Thus, crystallization degree was calculated from the following relation. $Crystallization degree \left(%\right) = \left(crystal portion integral diffracted intensities/total integral diffracted intensities\right) \times 100.$

Air permeability (cc / cm² /sec.): Measured according to the Frazir type method described in JIS-L-1096. More specifically, 3 specimens, each of 15 cm in length and 15 cm in width, were prepared. A Frazir type tester was used in such a way that, after a specimen was attached to one end of a cylinder, a suction pump adjustment was made by means of a variable resistor so as to allow an inclined type barometer to give a pressure reading of 12.7 mmH₂O. Then, the quantity of air passing through the specimen (cc/cm²/sec.) was determined on the basis of pressure readings of a vertical type barometer and according to the type of air spouting orifice used. Average value with respect to three specimens was taken as air permeability.

### Example 1

A polybutylene succinate (number-average molecular weight: 50,000) having a melting point of 116°C and an MFR value of 30 g/10 min., and containing 1 wt % of talc, was used. This polymer was melt spun through a circular spinneret at a spinning temperature of 190°C and at a mass out flow rate from each orifice of 0.67 g/min. Filaments spun were quenched by a conventional quenching device, and were then drafted and attenuated at a drafting speed of 2,000 m/min. Filaments were spread open each other and deposited on a collecting surface of a travelling conveyor, being thus formed into a web. The web was then passed through a partial bonding apparatus with heat and pressure comprising embossing rolls wherein partial bonding with heat and pressure was carried out under the following conditions: roll temperature of 90°C; and pressure bonded area ratio of 7.6 %. Thus, a filament nonwoven fabric comprised of filaments having a single filament fineness of 3.0 denier, with a weight per unit area of 60 g/m², was obtained. The constituent filaments of the web had a crystallization degree of 18 % and a supercool index of 0.41.

The filament nonwoven fabric obtained was preheated to 80°C and by using a mold the preheated nonwoven fabric was formed into a conical coffee filter having an opening diameter of 8.5 cm and a depth of 4.5 cm. This coffee filter was a good formed piece. The formed piece had an air permeability of 120 cc/cm² /sec. The formed filter was put into a continuous composting arrangement, and in about one month it had been composted leaving no trace of it.

### Example 2

An L-lactic acid / hydroxycaproic acid copolymer (number-average molecular weight: 90,000; weight ratio = 88/12) having a melting point of 162°C and an MFR value of 20 g/10 min., and containing 1 wt % of boron nitride, was used. This polymer was melt spun through a spinneret identical to the one used in Example 1 at a spinning temperature of 200°C and at a mass out flow rate from each orifice of 0.89 g/min. Filaments spun were quenched by a conventional quenching device, and were then drafted and attenuated at a drafting speed of 2,000 m/min. Filaments were spread open each other and deposited on a travelling conveyor, being thus formed into a web. The web was then passed through a partial bonding apparatus with heat and pressure comprising embossing rolls wherein partial bonding with heat and pressure was carried out under the conditions of roll temperature, 132°C, and pressure bonded area ratio, 6.5 %. Thus, a filament nonwoven fabric comprised of filaments having a single filament fineness of 4.0 denier, with a weight per unit area of 65 g/m², was obtained. The constituent filaments of the web had a crystallization degree of 21 % and a supercool index of 0.52.

The filament nonwoven fabric obtained was preheated to 120°C and was formed by pressing into a plant pot having an opening diameter of 10.5 cm and a depth of 5.5 cm. In this way, good formed piece was obtained. The formed plant pot had an air permeability of 170 cc/cm² /sec. A plant potted in this formed plant pot was set, together with the pot, for growth in the ground at an intended location. The plant smoothly grew into a mature tree. Three years after the plant in the plant pot was initially set in the ground, it was found that the plant pot had been degraded in the earth with no trace left of it.

### Examples 3 and 4

A copolymer of L-lactic acid / glycolic acid = 80 / 20 mol% having a melting point of 111°C, an MFR value of 30 g / 10 min. and a number average molecular weight of 70,000 was used as a low melting point component in Fig. 5, and a poly(D, L-lactic acid) of L-lactic acid/D-lactic acid = 90 / 10 mol% having a melting point of 141°C, an MFR value of 20 g/10 min. and a number average molecular weight of 90,000 was used as a high melting point component, the two components being used in the ratio of high melting point component / low melting point component = 1 / 1 by weight. The two components were melt spun through a spinneret having a nozzle configuration such that in a split type composite cross section as shown in Fig. 5, the low melting point component was disposed at the core side and the high melting point component at the leaf side, with a spinning temperature set at 170°C and a mass out flow rate from each orifice of 1.36 g/min. Filaments spun were quenched by a conventional quenching device, and were then drafted and attenuated at a drafting speed of 1,500 m/min., then spread open each other and deposited on a collecting surface of a travelling conveyor. Then, the filaments were subjected to temporary bonding with heat and pressure under the conditions of: embossing temperature, 51°C; linear pressure of a roll set, 10 kg/cm; pressure bonded area ratio, 6.5 %; and pressure bonded spot density, 36 bonded areas per cm², whereby a nonwoven web was formed. Then, the web was subjected to a three-dimensionally-entangling treatment by pressured liquid streams. That is, the nonwoven web was placed on a moving wire net (of 48 mesh) and exposed to jet streams of pressure liquid. For this purpose, an apparatus having orifices arranged in three rows, each orifice having a hole diameter of 0.2 mm and inter-hole spacing of 0.4 mm, was employed. For the pressure liquid, water was used. Two kinds of jet pressure were used, namely, 40 kg / cm² G × 4 times (Example 3), and 100 kg / cm² G × 4 times (Example 4). Excess water in the web was removed by means of mangle rolls, and then the web was dried. In Example 3, in which the jet pressure applied was 40kg/cm² G, the nonwoven fabric obtained was a three-dimensionally entangled nonwoven fabric, with temporary bonded areas with heat and pressure left unremoved. In Example 4, in which the jet pressure applied was 100 kg / cm² G, the nonwoven fabric obtained had constituent filaments thereof three-dimensionally entangled all over, with temporary bonded areas with heat and pressure completely separated. These nonwoven fabrics had a weight per unit area of 70. g/m². Their constituents filaments had a single-filament fineness of 3.5 denier, a crystallization degree of 16 %, and a supercool index of 0.6.

The filament nonwoven fabrics thus obtained were each preheated to 100°C and formed by pressing into a plant pot having an opening diameter of 10.5 cm and a depth of 5.5 cm. In this way, good formed pieces were obtained. The formed plant pots, of both Examples 3 and 4, had an air permeability of about 160 cc/cm² sec. A plant potted in each formed plant pot was set, together with the pot, for growth in the ground at an intended location. The plant smoothly grew into a mature tree. Three years after the plant in the plant pot was initially set in the ground, it was found that the plant pot had been degraded in the earth with no trace left of it.

## Claims

1. A nonwoven fabric made up of filaments comprised of a biodegradable polymer composed principally of a polylactic acid-based polymer or a polyalkylene dicarboxylate, wherein the filaments are partially bonded with heat and pressure or the filaments are three-dimensionally-entangled after partially bonded with heat and pressure and wherein the filaments have a crystallization degree of 7 to 40 % and a supercool index of 0.4 or more.

2. A nonwoven fabric as set forth in claim 1, wherein the biodegradable polymer comprises a polymer selected from the group consisting of poly(D-lactic acid), poly(L-lactic acid), copolymers of D-lactic acid and L-lactic acid, copolymers of D-lactic acid and hydroxy-carboxylic acid, and copolymers of L-lactic acid and hydroxy-carboxylic acid, or a blend of such polymers.

3. A nonwoven fabric as set forth in claim 1, wherein the biodegradable polymer is a polymer selected from the group consisting of polybutylene succinate, polyethylene succinate, polybutylene adipate, and polybutylene sebacate, or a copolymer in which such polymers are present as main repeating units.

4. A nonwoven fabric as set forth in claim 1, wherein the biodegradable polymer is added with a crystallizing agent.

5. A nonwoven fabric as set forth in claim 1, wherein the nonwoven fabric has spottedly fusion bonded areas such that individual filaments at partially preformed temporary bonded areas with heat and pressure are partially separated from one another by a three-dimensionally entangling treatment, and wherein individual filaments at other areas than the spottedly fusion bonded areas which are not fusion-bonded are three-dimensionally entangled together so as to be integrated as a whole.

6. A nonwoven fabric as set forth in claim 1, wherein individual filaments at partially preformed temporary bonded areas with heat and pressure are completely separated from one another by a three-dimensionally entangling treatment whereby they are three-dimensionally interlaced with one another so as to be integrated as a whole.

7. A nonwoven fabric as set forth in claim 1, wherein the nonwoven fabric is thermoformable.

8. A nonwoven fabric as set forth in claim 7, wherein the biodegradable polymer comprises a polymer selected from the group consisting of poly(D-lactic acid), poly(L-lactic acid), copolymers of D-lactic acid and L-lactic acid, copolymers of D-lactic acid and hydroxy-carboxylic acid, and copolymers of L-lactic acid and hydroxy-carboxylic acid, or a blend of such polymers, said polylactic acid-based polymer having a number-average molecular weight of from 50,000 to 95,000.

9. A method of fabricating a nonwoven fabric made up of filaments comprised of a biodegradable polymer composed principally of a polylactic acid-based polymer or a polyalkylene dicarboxylate, comprising the steps of melting the biodegradable polymer, said biodegradable polymer having a melt flow rate of 10 to 100 g/10 minutes as measured at 190°C according to ASTM-D-1238 (E), in a temperature range of from (Tm + 20)°C to (Tm + 80)°C, where Tm°C is the melting point of the biodegradable polymer; extruding the melt through a spinneret into filaments; drafting the extruded filaments by means of a suction device disposed below the spinneret under a quenching air blow generated through a conventional device and at a drafting speed of from 1,000 to 5,000 m/minute, thereby fining them down into finer filaments; then depositing such filaments, as they are spread open each other, and are laid up on a travelling collector surface to form a web; and heat-treating the web thereby to obtain the nonwoven fabric.

10. A fabricating method as set forth in claim 9, wherein the biodegradable polymer is a polymer selected from the group consisting of poly(D-lactic acid), poly(L-lactic acid), copolymers of D-lactic acid and L-lactic acid, copolymers of D-lactic acid and hydroxy-carboxylic acid, and copolymers of L-lactic acid and hydroxy-carboxylic acid, or a blend of such polymers.

11. A fabricating method as set forth in claim 9, wherein the biodegradable polymer is a polymer selected from the group consisting of polybutylene succinate, polyethylene succinate, polybutylene adipate, and polybutylene sebacate, or a copolymer in which such polymers are present as main repeating units.

12. A fabricating method as set forth in claim 9, wherein a crystallizing agent is added to the biodegradable polymer.

13. A fabricating method as set forth in claim 9, wherein constituent filaments of the web are partially bonded with heat and pressure at a temperature lower than the melting point of the biodegradable polymer.

14. A fabricating method as set forth in claim 13, wherein two or more kinds of components comprising said biodegradable polymer are melt spun into filaments by means of a spinneret which provides a composite sectional configuration with respect to the cross section of each of the filaments, and wherein said partial bonding with heat and pressure is effected at a temperature lower than the melting point of one of said two or more kinds of components which is lowermost of their melting points.

15. A fabricating method as set forth in claim 9, which further comprises subjecting the web to partial bonding with heat and pressure thereby to form temporary bonded areas with heat and pressure, then effecting a three-dimensionally entangling treatment with respect to the web thereby to cause individual filaments at the temporary bonded areas with heat and pressure to be at least partially separated, and three-dimensionally entangled individual filaments in the separated condition thereby to integrate filaments of the web as a whole.

16. A fabricating method as set forth in claim 15, wherein the step of partially bonding with heat and pressure for forming temporary bonded areas with heat and pressure is carried out by pressing the web by an embossing roll, said partial bonding with heat and pressure being effected at a processing temperature of from (Tm - 80)°C to (cm - 50)°C, where Tm°C is the melting point of one of the components of constituent filaments which is lowermost of the melting points of the components, with the linear pressure of the roll set within a range of from 10 to 100 kg/cm.

17. A fabricating method as set forth in claim 9, wherein the nonwoven fabric obtained is subjected to a thermoforming process.

18. A fabricating method as set forth in claim 9, wherein the biodegradable polymer comprises a polylactic acid-based polymer, said polylactic acid-based polymer being a polymer selected from the group consisting of poly(D-lactic acid), poly(L-lactic acid), copolymers of D-lactic acid and L-lactic acid, copolymers of D-lactic acid and hydroxy-carboxylic acid, and copolymers of L-lactic acid and hydroxy-carboxylic acid, or a blend of such polymers, said polylactic acid-based polymer having a number-average molecular weight of from 50,000 to 95,000.

19. A fabricating method as set forth in claim 9, wherein the drafting speed by the suction device during the process of drafting is 1,200 to 3,000 m/minute.

## Patentansprüche

1. Vliesstoff bestehend aus Filamenten, die ein biologisch abbaubares Polymer aufweisen, das sich hauptsächlich aus einem Polymilchsäure-basierten Polymer oder einem Polyalkylen-Dicarboxylat zusammensetzt, wobei die Filamente mit Wärme und Druck partiell verbunden werden oder die Filamente dreidimensional verschlungen werden, nachdem sie mit Wärme und Druck partiell verbunden wurden, und wobei die Filamente einen Kristallisationsgrad von 7 bis 40 % und einen Supercool-Index von 0,4 oder mehr aufweisen.

2. Vliesstoff nach Anspruch 1, **dadurch gekennzeichnet, dass** das biologisch abbaubare Polymer ein Polymer aus der Gruppe aufweist, die aus Poly-(D-Milchsäure), Poly-(L-Milchsäure), Copolymeren von D-Milchsäure und L-Milchsäure, Copolymeren von D-Milchsäure und Hydroxycarbonsäure, und Copolymeren von L-Milchsäure und Hydroxycarbonsäure, oder einer Mischung dieser Polymere besteht.

3. Vliesstoff nach Anspruch 1, **dadurch gekennzeichnet, dass** das biologisch abbaubare Polymer ein Polymer aus der Gruppe ist, die aus Polybutylensuccinat, Polyethylensuccinat, Polybutylenadipat und Polybutylensebacat, oder einem Copolymer, in dem diese Polymere als hauptsächliche Wiederholungseinheiten vorliegen, besteht.

4. Vliesstoff nach Anspruch 1, **dadurch gekennzeichnet, dass** dem biologisch abbaubaren Polymer ein Kristallisationsmittel zugesetzt ist.

5. Vliesstoff nach Anspruch 1, **dadurch gekennzeichnet, dass** der Vliesstoff punktuell schmelzverbundene Stellen aufweist, so dass einzelne Filamente an mit Wärme und Druck partiell vorgeformten temporär verbundenen Stellen durch eine dreidimensionale Verschlingungsbehandlung partiell voneinander getrennt werden, und wobei einzelne Filamente an anderen Stellen als den punktuell schmelzverbundenen Stellen, die nicht schmelzverbunden sind, dreidimensional zusammen verschlungen werden, um als Ganzes integriert zu werden.

6. Vliesstoff nach Anspruch 1, **dadurch gekennzeichnet, dass** einzelne Filamente an mit Wärme und Druck partiell vorgeformten temporär verbundenen Stellen durch eine dreidimensionale Verschlingungsbehandlung vollständig voneinander getrennt werden, wodurch sie dreidimensional miteinander verflochten werden, so dass sie als Ganzes integriert werden.

7. Vliesstoff nach Anspruch 1, **dadurch gekennzeichnet, dass** der Vliesstoff thermoformbar ist.

8. Vliesstoff nach Anspruch 7, **dadurch gekennzeichnet, dass** das biologisch abbaubare Polymer ein Polymer aus der Gruppe aufweist, die aus Poly-(D-Milchsäure), Poly-(L-Milchsäure), Copolymeren von D-Milchsäure und L-Milchsäure, Copolymeren von D-Milchsäure und Hydroxycarbonsäure, und Copolymeren von L-Milchsäure und Hydroxycarbonsäure, oder einer Mischung dieser Polymere besteht, wobei das Polymilchsäure-basierte Polymer ein Zahlenmittel-Molekulargewicht von 50.000 bis 95.000 hat.

9. Verfahren zur Herstellung eines Vliesstoffes bestehend aus Filamenten, die ein biologisch abbaubares Polymer aufweisen, das sich hauptsächlich aus einem Polymilchsäure-basierten Polymer oder einem Polyalkylen-Dicarboxylat zusammensetzt, welches folgende Schritte umfasst: das Schmelzen des biologisch abbaubaren Polymers, wobei das biologisch abbaubare Polymer eine Schmelzflussrate von 10 bis 100 g / 10 Minuten aufweist, gemessen bei 190 °C gemäß ASTM-D-1238 (E), in einem Temperaturbereich von (Tm + 20) °C bis (Tm + 80) °C, wobei Tm°C der Schmelzpunkt des biologisch abbaubaren Polymers ist; Extrudieren der Schmelze durch eine Spinndüse in Filamente; Verstrecken der extrudierten Filamente mittels einer unter der Spinndüse angeordneten Saugvorrichtung unter abschreckender Blasluft, die durch eine herkömmliche Vorrichtung erzeugt wird, und bei einer Verstreckungsgeschwindigkeit von 1.000 bis 5.000 m / Minute, wodurch sie in feinere Filamente verfeinert werden; dann Ablegen dieser Filamente, wie sie einander offen ausgebreitet werden, und auf eine laufende Sammleroberfläche aufgelegt werden, um eine Bahn zu bilden; und Wärmebehandeln der Bahn, um dadurch den Vliesstoff zu gewinnen.

10. Herstellungsverfahren nach Anspruch 9, **dadurch gekennzeichnet, dass** das biologisch abbaubare Polymer ein Polymer aus der Gruppe ist, die aus Poly-(D-Milchsäure), Poly-(L-Milchsäure), Copolymeren von D-Milchsäure und L-Milchsäure, Copolymeren von D-Milchsäure und Hydroxycarbonsäure, und Copolymeren von L-Milchsäure und Hydroxycarbonsäure, oder einer Mischung dieser Polymere besteht.

11. Herstellungsverfahren nach Anspruch 9, **dadurch gekennzeichnet, dass** das biologisch abbaubare Polymer ein Polymer aus der Gruppe ist, die aus Polybutylensuccinat, Polyethylensuccinat, Polybutylenadipat und Polybutylensebacat, oder einem Copolymer, in dem diese Polymere als hauptsächliche Wiederholungseinheiten vorliegen, besteht.

12. Herstellungsverfahren nach Anspruch 9, **dadurch gekennzeichnet, dass** dem biologisch abbaubaren Polymer ein Kristallisationsmittel zugesetzt ist.

13. Herstellungsverfahren nach Anspruch 9, **dadurch gekennzeichnet, dass** einen Bestandteil der Bahn bildende Filamente mit Wärme und Druck bei einer Temperatur, die niedriger als der Schmelzpunkt des biologisch abbaubaren Polymers ist, partiell verbunden werden.

14. Herstellungsverfahren nach Anspruch 13, **dadurch gekennzeichnet, dass** zwei oder mehr Arten von Komponenten, die das biologisch abbaubare Polymer aufweisen, mittels einer Spinndüse, die eine sektionale Verbundkonfiguration in Bezug auf den Querschnitt jedes der Filamente bereitstellt, zu Filamenten schmelzgesponnen werden, und wobei das partielle Verbinden mit Wärme und Druck bei einer Temperatur herbeigeführt wird, die niedriger als der Schmelzpunkt einer der zwei oder mehr Arten von Komponenten ist, der der niedrigste ihrer Schmelzpunkte ist.

15. Herstellungsverfahren nach Anspruch 9, das weiterhin umfasst, die Bahn einer partiellen Verbindung mit Wärme und Druck zu unterziehen, um dadurch mit Wärme und Druck temporär verbundene Stellen zu bilden, dann eine dreidimensionale Verschlingungsbehandlung in Bezug auf die Bahn herbeizuführen, um dadurch zu bewirken, dass einzelne Filamente an den mit Wärme und Druck temporär verbundenen Stellen mindestens partiell getrennt werden, und dreidimensional verschlungene einzelne Filamente im getrennten Zustand vorliegen, um dadurch Filamente der Bahn als Ganzes zu integrieren.

16. Herstellungsverfahren nach Anspruch 15, **dadurch gekennzeichnet, dass** der Schritt des partiellen Verbindens mit Wärme und Druck zum Bilden mit Wärme und Druck temporär verbundener Stellen ausgeführt wird, indem die Bahn durch eine Prägewalze gepresst wird, wobei das partielle Verbinden mit Wärme und Druck bei einer Verarbeitungstemperatur von (Tm - 80) °C bis (Tm - 50) °C herbeigeführt wird, wobei Tm °C der Schmelzpunkt einer der Komponenten von einen Bestandteil bildenden Filamenten ist, der der niedrigste der Schmelzpunkte der Komponenten ist, wobei der lineare Druck der Walze innerhalb eines Bereichs von 10 bis 100 kg / cm eingestellt wird.

17. Herstellungsverfahren nach Anspruch 9, **dadurch gekennzeichnet, dass** der gewonnene Vliesstoff einem Thermoformprozess unterzogen wird.

18. Herstellungsverfahren nach Anspruch 9, **dadurch gekennzeichnet, dass** das biologisch abbaubare Polymer ein Polymilchsäure-basiertes Polymer aufweist, wobei das Polymilchsäure-basierte Polymer ein Polymer aus der Gruppe ist, die aus Poly-(D-Milchsäure), Poly-(L-Milchsäure), Copolymeren von D-Milchsäure und L-Milchsäure, Copolymeren von D-Milchsäure und Hydroxycarbonsäure, und Copolymeren von L-Milchsäure und Hydroxycarbonsäure, oder einer Mischung dieser Polymere besteht, wobei das Polymilchsäure-basierte Polymer ein Zahlenmittel-Molekulargewicht von 50.000 bis 95.000 hat.

19. Herstellungsverfahren nach Anspruch 9, **dadurch gekennzeichnet, dass** die Verstreckungsgeschwindigkeit durch die Saugvorrichtung während des Verstreckungsprozesses 1.200 bis 3.000 m / Minute beträgt.

## Revendications

1. Etoffe non tissée consistant en filaments constitués d'un polymère biodégradable composé principalement d'un polymère à base d'acide polylactique ou d'un polyalkylène dicarboxylate, où les filaments sont partiellement liés grâce à la chaleur et à la pression ou bien les filaments sont entremêlés dans les trois dimensions après avoir été partiellement liés grâce à la chaleur et la pression et où les filaments présentent un degré de cristallisation de 7 à 40 % et un indice de super-refroidissement de 0,4 ou plus.

2. Etoffe non tissée selon la revendication 1, dans laquelle le polymère biodégradable comprend un polymère sélectionné parmi le groupe constitué de poly(acide D-lactique), de poly(acide L-lactique), de copolymères d'acide D-lactique et d'acide L-lactique, de copolymères d'acide D-lactique et d'acide hydroxycarboxylique, et de copolymères d'acide L-lactique et d'acide hydroxycarboxylique, ou d'un mélange de tels polymères.

3. Etoffe non tissée selon la revendication 1, dans laquelle le polymère biodégradable est un polymère sélectionné parmi le groupe constitué de polysuccinate de butylène, de polysuccinate d'éthylène, de polyadipate d'éthylène, et de polysébacate de butylène, ou d'un copolymère dans lequel de tels polymères sont présents en tant que principales unités qui se répètent.

4. Etoffe non tissée sont la revendication 1, dans laquelle le polymère biodégradable se voit ajouter un agent de cristallisation.

5. Etoffe non tissée selon la revendication 1, dans laquelle l'étoffe non tissée comporte des zones liées par fusion par points de sorte que les filaments individuels au niveau des zones liées temporairement préformées partiellement grâce à la chaleur et à la pression sont partiellement séparés les uns des autres par un traitement d'entremêlement dans les trois dimensions et dans laquelle les filaments individuels au niveau de zones autres que les zones liés par fusion de manière par points, qui ne sont pas liées par fusion, sont entremêlés dans les trois dimensions ensemble de manière à être intégrés en un tout.

6. Etoffe non tissée selon la revendication 1, dans laquelle les filaments individuels au niveau de zones temporairement liées préformées partiellement grâce à la chaleur et la pression sont complètement séparés les uns des autres par un traitement d'entremêlement dans les trois dimensions, grâce à quoi ils sont entrelacés dans les trois dimensions les uns les autres de manière à être intégrés en un tout.

7. Etoffe non tissée selon la revendication 1, dans laquelle l'étoffe non tissée est thermoformable.

8. Etoffe non tissée selon la revendication 7, dans laquelle le polymère biodégradable comprend un polymère sélectionné parmi le groupe constitué de poly(acide D-lactique), de poly(acide L-lactique), de copolymères d'acide D-lactique et d'acide L-lactique, de copolymères d'acide D-lactique et d'acide hydroxycarboxylique, et de copolymères d'acide L-lactique et d'acide hydroxycarboxylique ou un mélange de tels polymères, ledit polymère à base d'acide polylactique ayant un nombre de masse moléculaire moyen de 50 000 à 95 000.

9. Procédé de fabrication d'une étoffe non tissée consistant en filaments constitués d'un polymère biodégradable composé principalement d'un polymère à base d'acide polylactique ou d'un polyalkylène dicarboxylate, comprenant les étapes consistant à faire fondre le polymère biodégradable, ledit polymère biodégradable ayant une vitesse d'écoulement à l'état fondu de 10 à 100 g/10 min telle que mesurée à 190°C conformément à la norme ASTM-D-1238 (E) dans une plage de températures de (Tm + 20)°C à (Tm + 80)°C, où Tm°C est le point de fusion du polymère biodégradable, à extruder le bain de fusion au travers d'une filière en filaments, à étirer les filaments extrudés au moyen d'un dispositif d'aspiration disposé au-dessous de la filière sous un souffle d'air de trempe généré par le biais d'un dispositif classique et à une vitesse d'étirage de 1 000 à 5 000 m/min, en les affinant ainsi en filaments plus fins, à déposer ensuite les mêmes filaments, tels qu'ils sont étalés ouverts les uns aux autres, et sont disposés sur une surface de dispositif de recueil qui se déplace pour former un tissu, et à effectuer un traitement par la chaleur du tissu afin d'obtenir ainsi l'étoffe non tissée.

10. Procédé de fabrication selon la revendication 9, dans lequel le polymère biodégradable est un polymère sélectionné parmi le groupe constitué de poly(acide D-lactique), de poly(acide L-lactique), de copolymères d'acide D-lactique et d'acide L-lactique, de copolymères d'acide D-lactique et d'acide hydroxycarboxylique, et de copolymères d'acide L-lactique et d'acide hydroxycarboxylique, ou d'un mélange de tels polymères.

11. Procédé de fabrication selon la revendication 9, dans lequel le polymère biodégradable est un polymère sélectionné parmi le groupe constitué du polysuccinate de méthylène, du polysuccinate d'éthylène, du polyadipate de butylène, et du polysébacate de butylène, ou d'un copolymère dans lequel de tels polymères sont présents en tant que principales unités qui se répètent.

12. Procédé de fabrication selon la revendication 9, dans lequel un agent de cristallisation est ajouté au polymère biodégradable.

13. Procédé de fabrication selon la revendication 9, dans lequel les filaments constitutifs du tissu sont partiellement liés grâce à la chaleur et à la pression à une température inférieure au point de fusion du polymère biodégradable.

14. Procédé de fabrication selon la revendication 13, dans lequel deux ou plus types de composants constitués dudit polymère biodégradable sont filés par fusion en filaments au moyen d'une filière qui procure une configuration en coupe composite en ce qui concerne la section transversale de chacun des filaments, et dans lequel ladite liaison partielle grâce à la chaleur et à la pression est effectuée à une température inférieure au point de fusion de l'un desdits deux ou plus types de composants qui est le plus bas de leurs points de fusion.

15. Procédé de fabrication selon la revendication 9, qui comprend en outre lé fait de soumettre le tissu à une liaison partielle grâce à la chaleur et à la pression afin de former ainsi des zones temporairement liées grâce à la chaleur et à la pression, en effectuant ensuite un traitement d'entremêlement dans les trois dimensions par rapport au tissu afin d'amener ainsi les filaments individuels au niveau des zones temporairement liées grâce à la chaleur et à la pression à être au moins partiellement séparés, et les filaments individuels entremêlés dans les trois dimensions dans la condition séparée afin d'intégrer ainsi des filaments du tissu comme un tout.

16. Procédé de fabrication selon la revendication 15, dans lequel l'étape de liaison partielle grâce à la chaleur et à la pression pour former des zones temporairement liées grâce à la chaleur et à la pression est exécutée en pressant le tissu par le biais d'un rouleau de gaufrage, ladite liaison partielle grâce à la chaleur et à la pression étant effectuée à une température de traitement de (Tm - 80)°C à (Tm - 50)°C, où Tm°C est le point de fusion de l'un des composants des filaments constitutifs qui est le plus bas des points de fusion des composants, la pression linéaire de l'ensemble de rouleaux se trouvant dans une plage de 10 à 100 kg/cm.

17. Procédé de fabrication selon la revendication 9, dans lequel l'étoffe non tissée obtenue est soumise à un traitement de thermoformage.

18. Procédé de fabrication selon la revendication 9, dans lequel le polymère biodégradable comprend un polymère à base d'acide polylactique, ledit polymère à base d'acide polylactique étant un polymère sélectionné parmi le groupe constitué de poly(acide D-lactique), de poly(acide L-lactique), de copolymères d'acide D-lactique et d'acide L-lactique, de copolymères d'acide D-lactique et d'acide hydroxycarboxylique, et de copolymères d'acide L-lactique et d'acide hydroxycarboxylique, ou d'un mélange de tels polymères, ledit polymère à base d'acide polylactique ayant un nombre de masse moléculaire moyen de 50 000 à 95 000.

19. Procédé de fabrication selon la revendication 9, dans lequel la vitesse d'étirage du fait du dispositif d'aspiration au cours du traitement d'étirage est de 1 200 à 3 000 m/min.
